

P. A. E. ARMSTRONG.  
PROCESS FOR ELECTRIC WELDING.  
APPLICATION FILED MAR. 23, 1915.

1,241,900.

Patented Oct. 2, 1917.



Percy A. E. Armstrong, <sup>INVENTOR</sup>  
Prindle, Bright & Small, <sup>BY</sup> ATTORNEYS

# UNITED STATES PATENT OFFICE.

PERCY A. E. ARMSTRONG, OF NEW YORK, N. Y., ASSIGNOR TO WALTER L. CLARK AND ARTHUR H. ADAMS, A COPARTNERSHIP UNDER THE NAME OF THE QUASI-ARC COMPANY, OF NEW YORK, N. Y.

## PROCESS FOR ELECTRIC WELDING.

1,241,900.

Specification of Letters Patent.

Patented Oct. 2, 1917.

Application filed March 23, 1915. Serial No. 16,435.

To all whom it may concern:

Be it known that I, Percy A. E. Armstrong, of New York, in the county of New York and in the State of New York, have invented a certain new and useful Improvement in Processes for Electric Welding, and do hereby declare that the following is a full, clear, and exact description thereof.

My invention relates to processes, in which 10 an electric current is employed to fuse a metal electrode so that the fused metal is deposited upon a metal surface or surfaces which are thereby welded or patched.

The object of my invention has been to 15 provide such a process by which metal, such as manganese steel, which is capable of being treated by the application of fluids, such as water, may be so treated during the process of depositing it as aforesaid. More particularly, the object of my invention is to 20 provide such a process for so depositing manganese steel upon manganese steel which has been heat-treated that the metal being deposited shall also be heat-treated.

25 In the accompanying drawing,

The figure shows a form of apparatus being used in the practice of my said process.

In depositing manganese steel upon manganese steel which has been heat-treated, it 30 is frequently found that the original metal cracks soon after the deposit upon it of the fused metal, due to the heat being absorbed upon one face quicker than another, which sets up internal strains in the body which 35 have the effect of making cracks appear. Further, the deposited metal itself is frequently cracked, owing to the fact that the deposited metal has cooled or partly cooled prior to the appearance of the cracks and is 40 unable to accommodate itself to the movement producing the cracks.

To overcome these difficulties, I have conceived the idea of heat-treating the deposited metal as it is deposited and preventing the heat therefrom being transmitted to the casting. As is well known, manganese steel is made very tough and a high degree of tensile strength is developed in it by means of heat-treating; that is, 45 by heating it to a red heat and cooling in water, preferably very cold water. According to my invention, considered in its specific aspect as being applied to manganese steel, the deposited metal, while still

50 at a red heat, is cooled by means of a stream of fluid, preferably a stream of cold water, with the result of heat-treating the deposited metal and preventing the heat therefrom being transmitted into the casting. I find that this prevents the cracking of the 55 casting or other piece of work of manganese steel upon which the metal is being deposited, and it enables layer upon layer to be deposited, each layer being partially heat-treated as deposited and being thereby 60 given a high resistance to shock and tensile strain.

My process can be practised without the use of special apparatus, and in its simplest form it is only necessary to apply water to 70 the deposited metal as it is being deposited. It is more effective, however, to force the water upon the deposited metal in the form of a spray by means of compressed air. This is more beneficial than merely to use 75 water at less velocity, because each drop of water is thrown upon the surface with sufficient force to prevent the formation of a steam layer and it thereby more effectively acts upon the metal.

I prefer to use electrodes consisting of a metal core having a covering composed of a fusible slag so that the slag is melted and protects the molten metal from atmospheric action.

80 In the accompanying drawing I have shown such an electrode consisting of a metal core 1, having a slag covering 2. As a means for applying water to the deposited metal, I have shown a water pipe 3 having 85 an inclined, tapering nozzle 4, and an air pipe 5 having a tapering end 6 within, and at the same inclination as the nozzle 4, so that the air will force the water out of the nozzle 4 in the form of a spray. In the 90 specific instance shown in the drawing, the electrode was first touched to the manganese steel casting 7 near the left hand end of its upper surface, as seen in the figure, thus making an actual contact therewith, and 95 the current thus started. The electrode was then raised so as to be out of actual contact with the work but in actual contact with the molten metal and slag which were fused from the electrode by the current, and then 100 the electrode was moved gradually to the right, the water being sprayed upon the 105 deposited metal at the same time. The slag

floats upon the top of the deposited metal and protects it from the atmosphere, and the water quickly cools and solidifies both the deposited metal and the slag. I find 5 that this water treatment renders it easier to remove the slag from the deposited metal when the latter has cooled.

While I have illustrated my process by the best manner of practising the same 10 known to me, and by the use of the most effective and convenient apparatus for that purpose, which I have devised, I wish it to be understood that I claim the practising of my process for any purpose and with any 15 materials to which it is applicable, and that I regard my illustrated apparatus as typical only of many possible forms of apparatus which can be used for that purpose.

My invention not only contemplates the 20 use of an electrode having a manganese steel core, but of an electrode having a steel or manganese steel core, and having manganese in the insulating coating thereof. This latter form of an electrode is the subject of a 25 separate application for patent.

I claim:

1. The process of depositing metal by means of an electric current, which comprises connecting the work and a metal electrode with opposite poles of a source of electricity, said electrode being coated with insulating material that is adapted to act as a slag when fused, causing the current to flow between the end of the electrode and the 30 work, forming molten metal, and maintaining the electrode in actual touch with the molten metal, but out of actual contact with the work, and cooling the deposited metal as it is deposited, by the application of a cooling 35 fluid thereto.

2. The process of depositing metal by means of an electric current, which comprises connecting the work and a metal electrode with opposite poles of a source of electricity, said electrode being coated with insulating material that is adapted to act as a slag when fused, causing the current to flow between the end of the electrode and the work, forming molten metal, and maintaining the electrode in actual touch with the molten metal, but out of actual contact with the work, and cooling the deposited metal as it is deposited, by the application of water thereto.

55 3. The process of depositing metal by means of an electric current, which comprises connecting the work and a metal electrode with opposite poles of a source of electricity, said electrode being coated with insulating material that is adapted to act as a slag when fused, causing the current to flow between the end of the electrode and the work, forming molten metal, and maintaining the electrode in actual touch with 60 the molten metal, but out of actual contact

with the work, and cooling the deposited metal as it is deposited, by the application of a forceful spray of water thereto.

4. The process of depositing metal by means of an electric current, comprising 70 connecting the work and an electrode with opposite poles of a source of electricity and melting said electrode, and applying to the deposited metal a fluid adapted to change its character.

5. The process of depositing manganese steel upon a body of metal which consists in melting said steel at a high temperature and depositing it upon said body of metal, and immediately cooling the deposited metal by 80 applying a cooling agent thereto.

6. The process of depositing manganese steel upon work consisting of manganese steel, by means of an electric current, which comprises connecting the work and an electrode with opposite poles of a source of electricity, said electrode being coated with insulating material that is adapted to act as a slag when fused, said electrode comprising steel and manganese, melting the electrode 85 and thus depositing manganese steel upon the work, and applying a cooling fluid to the deposited metal.

7. The process of depositing manganese steel upon work consisting of manganese steel, by means of an electric current, which comprises connecting the work and an electrode with opposite poles of a source of electricity, said electrode being coated with insulating material that is adapted to act as a 95 slag when fused, said electrode comprising steel and manganese, melting the electrode and thus depositing manganese steel upon the work and applying cooling water to the deposited metal.

8. The process of depositing manganese steel upon work consisting of manganese steel, by means of an electric current, which comprises connecting the work and an electrode with opposite poles of a source of electricity, said electrode being coated with insulating material that is adapted to act as a 100 slag when fused, said electrode comprising steel and manganese, melting the electrode and thus depositing manganese steel upon the work and applying cooling water in the 105 form of a spray to the deposited metal.

9. The process of depositing manganese steel upon work consisting of manganese steel, by means of an electric current, which 110 comprises connecting the work and an electrode with opposite poles of a source of electricity, said electrode being coated with insulating material that is adapted to act as a slag when fused, said electrode comprising steel and manganese, melting the electrode 115 and thus depositing manganese steel upon the work and applying cooling water by means of a jet of compressed air to the deposited metal.

10. The process of depositing manganese steel by means of an electric current which consists in connecting the work and an electrode containing manganese steel, with opposite poles of a source of electricity, melting the electrode upon the work, and applying a cooling fluid to the deposited metal.
- 5 11. The process of depositing a metal by means of an electric current which consists in connecting the work and an electrode containing such metal with opposite poles of a source of electricity, melting the electrode
- 10 upon the work, and applying a cooling agent to the deposited metal.
12. The process of depositing a metal of high fusing point which consists in melting the same upon the work, and applying a cooling agent to the deposited metal.
- In testimony that I claim the foregoing I have hereunto set my hand.
- PERCY A. E. ARMSTRONG.

Witnesses:

MARIAN I. DEMPSEY,  
J. FREUDENVOLL.